

R. M. HARRINGTON.

METHOD OF PRODUCING LEAD SALTS.

APPLICATION FILED SEPT. 27, 1917.

1,308,948.

Patented July 8, 1919.



INVENTOR

RALPH M. HARRINGTON

BY

Herbert H. Thompson

ATTORNEY

# UNITED STATES PATENT OFFICE.

RALPH M. HARRINGTON, OF BROOKLYN, NEW YORK, ASSIGNOR TO ELMER A. SPERRY,  
OF BROOKLYN, NEW YORK.

## METHOD OF PRODUCING LEAD SALTS.

1,308,948.

Specification of Letters Patent. Patented July 8, 1919.

Application filed September 27, 1917. Serial No. 193,415.

To all whom it may concern:

Be it known that I, RALPH M. HARRINGTON, a citizen of the United States of America, residing at Brooklyn, in the county of 5 Kings and State of New York, have invented certain new and useful Improvements in Methods of Producing Lead Salts, of which the following is a specification.

This invention relates to an improved 10 method of making lead compounds electrolytically. More specifically it relates to the manufacture of compounds containing lead salts such as lead chromate, lead sulfate or lead carbonate by an electrolytic method.

15 I am aware that lead compounds have been produced, heretofore, by passing an electric current from a lead anode to a cathode through an anolyte capable of yielding a lead solvent and containing a soluble 20 carbonate, and a similar catholyte and then carbonating the anolyte by adding carbon dioxide and causing the desired product to be precipitated in the anolyte. I am also aware that it has been proposed to separate 25 the anolyte and catholyte by means of a diaphragm in order to prevent lead compounds from reaching the cathode. Certain objections have appeared in manufacturing, according to this method, which have seriously 30 limited its commercial exploitation.

By introducing the carbon dioxide, or other acid radical, into the catholyte, however, very important advantages are gained. For the sake of simplicity I will confine the 35 following disclosure to a method of manufacturing white lead although other lead compounds may be produced by the same method by using acid radicals other than carbon dioxide, such as sulfuric or chromic 40 acid, for example. The advantages, above referred to, may best be set forth by considering certain of the actions of the above described old method.

In this prior process the action is substantially as follows: Assuming that sodium acetate solution is used as the anolyte, lead acetate is formed at the anode. The carbonate in the anolyte reacts on the lead acetate to form white lead and obviously if the anolyte 50 is high in carbonate the white lead is formed on and adheres to the anode thus seriously interfering with the operation of the system. Thus, with this old method, it is necessary to keep the anolyte low in carbonate and

with this low concentration the anolyte is a 55 poor absorber of carbon dioxide.

In my process I pass the carbon dioxide into the catholyte which is made strongly alkaline so that the above objection is avoided. The strongly alkaline catholyte 60 readily absorbs the desired amount of carbon dioxide even though the latter is in dilute form as for example in flue gas. Preferably the catholyte should be at least fifty times stronger than the anolyte in alkalinity. 65

Under uniform conditions of temperature and current density the composition of both anolyte and catholyte remains practically constant, the rate of diffusion of the carbonate through the diaphragm being the 70 same as the rate of formation inside the cathode compartment. Thus the percentage of carbonate in the anolyte and also the product are under absolute control in my process which are very important advantages. 75

It is also old in the art to produce white lead by use of an electrolytic bifluid cell, i. e. one in which the catholyte and anolyte are kept separate by a diaphragm, and in which 80 a solution of lead salt is formed in the anolyte. In this process the anolyte and alkaline catholyte are withdrawn from the cell and mixed to produce lead hydroxid which is carbonated (outside the cell) to 85 precipitate white lead. Or, as an alternative, the catholyte and anolyte are withdrawn, the catholyte is then carbonated and the two then mixed to precipitate the white 90 lead outside the cell.

Both of the last two described processes are open to many objections, among which are the following. The process is not continuous. Furthermore provision must be made to prevent diffusion of the two fluids 95 in the cell. The lead in solution in the anolyte increases to such a high value that there is danger of it depositing on the cathode unless special precautions are taken.

On the other hand in my process the product is precipitated in the anolyte and the action is continuous. My process will be found to combine the advantages of the above mentioned old processes and to be free from the disadvantages and objections 100 thereof.

Other objects and advantages will appear as the invention is hereinafter developed.

Although my method is independent of the particular details of apparatus employed I have found the apparatus illustrated diagrammatically in the drawing to be very 5 convenient in carrying out the process.

Referring to the drawing it will be seen that a tank, or other fluid container, is provided. This tank is shown as containing an anode plate 2 and a frame 4. The frame 4, 10 has mounted on each side thereof a suitable diaphragm 5, 5, such as parchment paper or vegetable parchment, forming a compartment for and containing the cathode 3 and catholyte. The diaphragms 5, 5 permit only 15 a slow interchange of liquids by osmosis, and prevent solids passing therethrough.

The anode is a lead plate while the cathode may be of any conducting material such as iron, copper, etc. The tank 1 also 20 contains the anolyte and the frame 4 the catholyte. Although I have shown but one anode, cathode and frame a plurality may be provided if desired. The tank 1 is shown as provided with a downwardly tapering portion 6 connected by means of a pipe 7 to a settling tank 8 which in turn is provided with a pipe 10, at its upper portion, which terminates at the top of the tank 1. By operating a pump 9 shown in pipe line 7 the 25 anolyte in tank 1 may be circulated in the following path: from tank 1, through pipe 7 into settling tank 8 and through pipe 10 to the tank 1. Obviously any precipitate in the anolyte will settle to the bottom of tank 30 8 and may be drawn off through the cock or valve 11 provided for that purpose. Furthermore by circulating the anolyte, it is kept uniform throughout.

Means are also shown for circulating the 40 catholyte solution. A pipe 12 terminates at one end and near the bottom of frame 4 and at its other end at the bottom of a carbonating tower 16. A pipe 13 connects the upper part of frame 4 and the upper part of the 45 carbonating tower 16. A pump 15 is placed in line 12 to circulate the catholyte along the following path: from frame 4, through pipe 13, down through tower 16 and then through pipe 12 to the bottom of the frame 4. The 50 rate of circulation of the catholyte through the tower 16 may be controlled by a valve 14 in pipe 12 or by means of a valve 17 located in a by-pass 18 around the tower. The carbon dioxide is introduced through pipe 19 55 and travels upwardly, through a quantity of coke, 25 or the like which may be provided in the tower, and then exhausting at 24.

Flue gas contains carbon dioxide and may 60 therefore be used in carbonating the catholyte. Before introducing this gas through pipe 19 I prefer to purify it by passing it through a scrubber 20 charged with limestone 26 or like substance and through which a current of water is passed from pipe 21 to 65 pipe 22. The flue gas enters through pipe

23 at the bottom of scrubber 20, passes upwardly and is thereby purified and leaves by pipe 19.

The anolyte employed is a solution of an alkali metal salt, capable of yielding a lead 70 solvent; for example, sodium acetate. If desirable a small amount of soluble carbonate, such as sodium carbonate, or a small amount of lead acetate may be added.

The catholyte solution comprises the same 75 alkali metal salt; for example, sodium acetate, as the anolyte and in addition preferably contains a soluble carbonate, or hydrate or mixture of these. Thus sodium carbonate or bi-carbonate may be employed. The 80 catholyte, as mentioned before, is made more strongly alkaline than the anolyte.

Assuming that the above suggested compounds are employed, that a source of E. M. F. is connected across the plates, that flue 85 gas is supplied at 23 and that both the catholyte and anolyte are circulating the action is probably as follows:

The sodium acetate reacts with the lead plate to form lead acetate. Thus: 90



At the cathode, sodium reacts with water to form sodium hydroxid, thus:



The sodium hydroxid reacts with the carbon dioxide, in the carbonating tower 16, to form more or less sodium carbonate, thus:



The sodium carbonate thus formed in the catholyte reaches the anolyte by diffusing through the diaphragms 5, or by overflowing, and reacts with lead acetate to precipitate white lead, thus: 105



The white lead is precipitated in the anolyte by such a dilute solution of sodium carbonate that there is no danger of it adhering to the anode surface. 110

It will be noted, on inspection of the last equation, that sodium acetate is regenerated, 115 so that the process is not only continuous but also cyclic. The only materials consumed are water, carbon dioxide (flue gas) and lead. The precipitated white lead will settle in tank 8 and may be drawn off at 11. 120

In order to produce white lead similar to that produced by the "Dutch process" both large and small particles must be produced. Electrolytic white lead comparatively low in carbonate consists of very fine amorphous 125 particles while that comparatively high in carbonate consists of much larger more or less crystalline particles. A proper combination of these gives a white lead of minimum oil absorption and high covering 130

power. Thus by regulating the amount of carbon dioxid supplied to the catholyte the character and quality of the product may be controlled. This regulation may be effected 5 either by adjusting the valve 14 or the valve 17 either of which will control the amount of catholyte subjected to the carbon dioxid.

Having described my invention what I desire to secure by Letters Patent is:

10 1. The method of producing a lead compound electrolytically which comprises passing an electric current from a lead anode to a cathode through an electrolyte capable of yielding a lead solvent, substantially excluding lead compounds from said cathode by a diaphragm and introducing into the catholyte an acid capable of yielding an insoluble precipitate with lead when it reaches the anolyte within the cell.

20 2. The method of producing a lead compound electrolytically which comprises producing an alkaline hydrate at the cathode, at least partially neutralizing this hydrate by an acid capable of yielding an insoluble precipitate with lead and introducing the alkali salt thus formed into the anolyte within the cell.

30 3. The method of producing a lead compound electrolytically which comprises producing an alkaline hydrate at the cathode, at least partially neutralizing this hydrate by an acid capable of yielding an insoluble precipitate with lead and introducing the alkali salt thus formed into the anolyte to an extent substantially necessary to prevent lead forming in solution.

40 4. The method of producing a lead compound electrolytically which comprises producing an alkali hydrate at the cathode, at least partially neutralizing this hydrate by an acid capable of yielding an insoluble precipitate with lead, and introducing the alkali salt thus formed into the anolyte within the cell at substantially the same rate at which it forms in the catholyte.

50 5. The method of producing a lead compound electrolytically which comprises producing an alkaline hydrate at the cathode, at least partially neutralizing this hydrate by an acid capable of yielding an insoluble precipitate with lead, thus producing an alkali salt, precipitating the desired lead compound in the anolyte within the cell by introducing the alkali salt into the latter, circulating the anolyte and removing the precipitate from the anolyte at a place exterior to the electrolytic cell.

60 6. The method of producing a lead compound electrolytically which comprises producing an alkaline hydrate at the cathode, circulating the catholyte, introducing an acid radical into said catholyte exteriorly to the cell and introducing the alkali salt thus formed into the anolyte within the cell.

65 7. The method of producing white lead

electrolytically which comprises producing an alkaline hydrate in the catholyte, carbonating the hydrate in the catholyte to form an alkali carbonate, precipitating the white lead in the anolyte within the cell by introducing the carbonate into the anolyte and substantially excluding lead compounds from the cathode by means of a diaphragm.

8. The method of producing white lead electrolytically which comprises producing an alkaline hydrate at the cathode, carbonating the alkaline hydrate in the catholyte and introducing the alkali carbonate thus formed into a weakly alkaline or neutral anolyte by osmosis.

9. The method of producing white lead electrolytically which comprises producing an alkaline hydrate in a comparatively strongly alkaline catholyte, carbonating the alkaline hydrate in the catholyte and introducing the alkali carbonate thus formed into a comparatively weakly alkaline anolyte by osmosis.

10. The method of producing white lead electrolytically which comprises producing an alkaline hydrate in a comparatively strongly alkaline catholyte, carbonating the alkaline hydrate in the catholyte and introducing the alkali carbonate thus formed into a comparatively weakly alkaline anolyte through a diaphragm, the catholyte being maintained at least fifty times more strongly alkaline than the anolyte.

11. The method of forming a lead salt away from the surface of the lead anode of a bifluid electrolytic cell which comprises dissolving the anode and precipitating the lead salt by introducing the precipitating reagent first into the catholyte and then into the anolyte by osmosis.

12. The method of forming a lead salt away from the surface of the lead anode of a bifluid electrolytic cell which comprises dissolving the anode and precipitating the lead salt by introducing the precipitating reagent first into the catholyte and then into the anolyte through a diaphragm.

13. The method of producing a precipitate in the anolyte of a bifluid electrolytic cell which comprises introducing the precipitating agent from the catholyte, by osmotic action into the anolyte.

14. In apparatus for the production of white lead by electrolysis, a container adapted to contain a lead anode and a metallic cathode, a parchment compartment therein to separate the catholyte from the anolyte, a settling tank for the white lead precipitate, means for continuously circulating the anolyte through the container and tank, a mixing chamber, a source of supply of a gaseous acid radical for supplying said gas to said chamber and means for continuously circulating the catholyte through said compartment and chamber.

15. In apparatus for the production of white lead by electrolysis, a container adapted to contain a lead anode and a metallic cathode, a parchment compartment therein to separate the catholyte from the anolyte, a settling tank for the white lead precipitate, means for continuously circulating the anolyte through the container and tank, a mixing chamber, a source of supply of a gaseous acid radical for supplying said gas to said chamber, means for continuously circulating the catholyte through said compartment and chamber and a regulatable by-pass around said chamber.
16. The method of forming white lead away from the surface of the lead anode of a bifluid electrolytic cell which consists in circulating the anolyte around a path through and exterior to the cell, collecting the white lead exterior to the cell, circulating the catholyte around a separate similar path and introducing the acid radical to said catholyte exterior to the cell.
17. The method of producing white lead electrolytically which comprises producing

an alkaline hydrate at the cathode, carbonating the alkaline hydrate in the catholyte and introducing the alkali carbonate thus formed into a weakly alkaline anolyte through a diaphragm, the rate of carbonating being so proportioned that the white lead is precipitated between the anode and diaphragm.

18. The method of producing white lead electrolytically which comprises producing an alkaline hydrate at the cathode, carbonating the alkaline hydrate in the catholyte and introducing the alkali carbonate thus formed into a weakly alkaline anolyte by osmosis, the rate of carbonating being so proportioned that the white lead is precipitated between the anode and diaphragm, and the carbonate passes through the diaphragm at substantially the same rate as formed whereby the composition of the electrolyte remains substantially constant.

In testimony whereof I have affixed my signature.

RALPH M. HARRINGTON.